

July 3, 1934.

F. R. KEMMER

1,964,853

METHOD OF TREATING METAL POWDER

Filed April 7, 1933



FRANK R. KEMMER,

BY

*H.C. Biemann*  
ATTORNEY.

## UNITED STATES PATENT OFFICE

1,964,853

## METHOD OF TREATING METAL POWDER

Frank R. Kemmer, Larchmont, N. Y., assignor  
to Magnesium Products, Inc., Wilmington, Del.,  
a corporation of Delaware

Application April 7, 1933, Serial No. 664,933

24 Claims. (Cl. 75—17)

This invention relates to the production of metallic magnesium and more particularly to the recovery of the metal in coherent form from a powder containing the same.

5 In my copending application Serial #542,104, dated June 4, 1931, and entitled "Method of producing magnesium" I have described a process in which magnesium oxide ore and carbon are caused to react to form magnesium vapors which 10 are condensed to powder and the powder then treated in a rotary furnace for the production of molten metal. The present application is a continuation in part of the aforesaid application and resides in further developments in that phase of 15 the process described in my original application which is intended to result in a greater and more effective production of coherent metal from the powder.

More particularly, the present invention is designed to protect the magnesium powder before and during the treatment and to provide a treatment which will increase the amount of liquid metal which is obtained from the powder. This results not only in greater efficiency of conversion 25 into salable metal, but also decreases the amount of material remaining and which ordinarily is returned to the smelting furnace for reworking.

The present invention may be conducted in a number of ways. If a material of the character described in my co-pending application, Serial 30 #664,932, filed April 7, 1933, entitled "Method of and apparatus for condensing magnesium", is utilized, the procedure in the present case resides in taking the product which consists of a mixture 35 of magnesium powder and a protective liquid, which is ordinarily a hydrocarbon oil. The oil which protects the magnesium from oxidation while in storage, is separated from the powder, but of course leaving the particles of magnesium powder coated with a thin film of oil. The material 40 is charged into a rotary furnace, which is heated to a suitable temperature above the melting point of metallic magnesium and usually below the boiling point at the pressure used. At the same 45 time the material is subjected to a frictional action which may be obtained by rotation of the furnace and the consequent rubbing of the particles on each other and against the walls and the electrodes of the furnace. In addition thereto or 50 in lieu thereof, other mechanical means for producing this rubbing action may be used.

Because of the presence of the oil at the temperature used for the treatment there is vaporization and in some cases decomposition thereof, 55 which has three principal effects. First it drives

out of the apparatus any deleterious gases, such as air, which may be present, and thus prevents a change from the metallic condition to that of compounds of magnesium such as oxide, nitride, etc. Second, it prevents access of such gases by 60 maintaining a slight positive gas pressure in the apparatus. Third, it provides a reducing atmosphere which may have a beneficial effect in removing combined oxygen, if such exists, from the material being treated. Liquid magnesium is produced in the apparatus and it may be removed 65 therefrom as desired.

If a magnesium powder produced in another manner is used which does not contain oil, or other protective liquid, but is a finely divided dry powder, 70 the same is stored in an air tight container so as to prevent oxidation or other deterioration thereof. Any air or deleterious vaporizable substances are removed therefrom by means of a vacuum pump. In most cases it is preferable to replace the gases 75 removed from the magnesium powder by a gas or even a vaporizable liquid or solid, which is inert in the subsequent rotary furnace operation. The magnesium powder, thus protected, is then charged into a rotary furnace where it is heated 80 to the proper temperature as explained above and subjected to the rotating action or other action to give friction or rubbing for the production of liquid magnesium. In this case it is desirable, though not essential, to maintain the rotary furnace under at least a partial vacuum and in most 85 cases to have the gas remaining in the apparatus of an inert, or reducing character. The vacuum causes vaporization of magnesium, which may be condensed to give purified magnesium. In this 90 case there are combined two treatments, first a rubbing or frictional action producing crude liquid magnesium and, second, the refining thereof by distillation. Thus, I obtain purified magnesium directly from the powder by a single operation. 95 This results in a higher efficiency of recovery of metal from the powder than when the powder is distilled without the rubbing action.

In the accompanying drawing constituting a part hereof and in which like reference characters indicate like parts:

Figure 1 is an elevational view, partly diagrammatic in character, showing one embodiment of the present invention;

Figure 2 is a similar view of a modified form 105 thereof, and

Figure 3 is a fragmentary view of a slight modification of the system of Figure 2.

Referring to Figure 1, there is provided a storage receptacle 1 for a mixture of magnesium pow- 110

der and oil. By means of suitable transfer apparatus 2, the mixture is introduced into suitable apparatus 3 for the separation of the oil from the magnesium powder, as by sedimentation, centrifugal action or filtration. The magnesium powder 5 is introduced through the double vacuum valve 4, through duct 6 provided with a pressure relief valve 7, into a rotary inclined furnace 8. The furnace is provided with bands 9, resting on rollers 10 and suitable means, not shown, is provided for rotating the furnace at the desired speed. Along the inner periphery of the furnace is a series of longitudinal electrodes 11, extending out through the ends of the furnace and being connected with 15 suitable rings whereby electric current may be passed through the electrodes to provide the proper temperature within the furnace. A spout 12, as is well known, is provided at the discharge end of the furnace, the opening 13 being closed 20 by suitable means, which allows liquid to pass out onto spout 12. The liquid magnesium 14 is received in ladle 15.

In the operation of the invention the magnesium powder containing some small amount of oil is heated in the rotary furnace to a temperature above the melting point of metallic magnesium, but below the boiling point and the furnace is rotated so as to give a rubbing action of the particles on each other and on the walls of 30 the furnace. The electrodes, which provide the necessary heat, move continuously through the powder and further subject the powder to frictional action. The heat vaporizes the oil, which forces out any air in the apparatus through the 35 pressure relief valve 7. The atmosphere thus created is somewhat above atmospheric pressure, and therefore, prevents access of air. The atmosphere is of reducing character and assists in the reduction of magnesium oxide, if some of this 40 compound is present with the magnesium powder. As the magnesium assumes the liquid state, it is discharged through spout 12 and into chill car 15.

Referring to the modification shown in Figure 2, dry magnesium powder is placed in a storage 45 bin 16, provided with a double vacuum valve 17 for the introduction of material and a similar double vacuum valve 18 for the discharge of the material. A pipe 19 is provided with a valve 20, and is connected with a vacuum pump, not shown. 50 Another pipe 21 provided with a valve 22, allows the introduction into container 16 of a suitable gas, liquid or solid. Secured to the bottom of container 16 is duct 6' which in turn is connected to the inlet end of rotary furnace 8'. In this 55 modification the discharge end of the furnace is provided with an opening closed by a suitable airtight cover 23 and the spout 12' is placed in proximity to the lower end of the said furnace. A vacuum relief valve 24 is provided in duct 6'.

60 In the operation of the invention, the magnesium powder in container or bin 16 is first subjected to a vacuum to draw out all gases and vapors therefrom after which valve 20 is closed and valve 22 is opened, allowing the introduction 65 of a suitable gas or liquid which is inert at the temperature of operation of the rotary furnace. Among such materials are hydrocarbon gases or readily volatile liquids, hydrogen, helium and various others. The gas replaces the voids in the 70 evacuated powder, which is then discharged by means of valve 18 through duct 6' into furnace 8'. The furnace is heated and rotated as described above causing liquefaction of the magnesium by the action of the heat and friction. The inert or 75 reducing gas present acts to protect the mag-

nesium from oxidation. The degree of vacuum in the furnace 8' may be of any desired character. After the operation is completed relief valve 24 is opened to break the vacuum and the sealing device 23 is removed from the opening allowing 80 liquid metal to flow into the chill car 14'.

Although I have described my invention setting forth two specific embodiments thereof, the invention is not limited thereto as the examples given are intended to illustrate the invention and not to define the limits thereof. It is very apparent that other types of magnesium powder may be treated in the manner above set forth and the exact order of the steps given may be varied widely. It is possible to make various combinations of the steps outlined or to add other steps and to make various other changes without departing from the principles herein set forth. For instance, in place of valve 24, there may be connected in the system as shown in Figure 3 a condenser 25, and a vacuum pump 26 may be attached thereto to draw vapors of magnesium from furnace 8' into the condenser to give refined metal. A valve 27 may be placed in the system. Or a stream of inert gas may be used in place of a vacuum for this purpose. A vacuum is not essential in this modification as the magnesium powder may be heated in the furnace to above its normal boiling point and the vapors condensed with or without the aid of a protective gas. My 100 invention is therefore to be construed broadly and not to be limited except as expressed in the appended claims.

What I claim is:

1. A method of treating magnesium powder 110 which comprises mixing therewith a material capable of protecting the magnesium from combining with deleterious substances by preventing access thereof, and subjecting said powder to a temperature above the melting point and below 115 the boiling point of magnesium and to a rubbing action to cause magnesium particles to coalesce to form liquid metal.

2. A method of treating magnesium powder 120 which comprises mixing therewith a material capable of protecting the magnesium from combining with deleterious substances by preventing access thereof, subjecting said powder to a temperature above the melting point and below the boiling point of magnesium and to a rubbing 125 action to cause magnesium particles to coalesce to form liquid metal and preventing access of detrimental gases during said rubbing operation.

3. A method of treating magnesium powder 130 which comprises mixing therewith a gaseous material capable of protecting the magnesium from combining with deleterious substances by preventing access thereof, and subjecting said powder to a temperature above the melting point and below the boiling point of magnesium and to a 135 rubbing action to cause magnesium particles to coalesce to form liquid metal.

4. A method of treating magnesium powder 140 which comprises mixing therewith a liquid material capable of protecting the magnesium from combining with deleterious substances by preventing access thereof, and subjecting said powder to a temperature above the melting point and below the boiling point of magnesium and to a rubbing 145 action to cause magnesium particles to coalesce to form liquid metal.

5. A method of treating magnesium powder 150 which comprises subjecting the same to at least a partial vacuum, mixing therewith a material capable of protecting the magnesium from com-

- bining with deleterious substances by preventing access thereof, and subjecting said powder to a temperature above the melting point and below the boiling point of magnesium and to a rubbing action to cause magnesium particles to coalesce to form liquid metal. 5
6. A method of treating magnesium powder which comprises subjecting the same to at least a partial vacuum, mixing therewith a gaseous material capable of protecting the magnesium from combining with deleterious substances by preventing access thereof, and subjecting said powder to a temperature above the melting point and below the boiling point of magnesium and to a rubbing action to cause magnesium particles to coalesce to form liquid metal. 10
7. A method of treating magnesium powder which comprises mixing therewith a gaseous material capable of protecting the magnesium from combining with deleterious substances by preventing access thereof, subjecting said powder to a temperature above the melting point and below the boiling point of magnesium and to a rubbing action to cause magnesium particles to coalesce to form liquid metal, and providing a pressure during said rubbing operation sufficient to prevent access of air. 15
8. A method of treating magnesium powder which comprises mixing therewith a gaseous material capable of protecting the magnesium from combining with deleterious substances by preventing access thereof, subjecting said powder to a temperature above the melting point and below the boiling point of magnesium and to a rubbing action to cause magnesium particles to coalesce to form liquid metal, and providing a pressure during said rubbing operation by the heating and consequent expansion of said gaseous material sufficient to prevent access of air. 20
9. A method of treating magnesium powder which comprises mixing therewith a liquid material capable of protecting the magnesium from combining with deleterious substances by preventing access thereof, subjecting said powder to a temperature above the melting point and below the boiling point of magnesium and to a rubbing action to cause magnesium particles to coalesce to form liquid metal, and providing a gas pressure during said rubbing operation sufficient to prevent access of air. 25
10. A method of treating magnesium powder which comprises mixing therewith a liquid material capable of protecting the magnesium from combining with deleterious substances by preventing access thereof, subjecting said powder to a temperature above the melting point and below the boiling point of magnesium and to a rubbing action to cause magnesium particles to coalesce to form liquid metal, and providing a gas pressure during said rubbing operation sufficient to prevent access of air, by the heating and consequent vaporization of at least part of said liquid material. 30
11. A method of treating magnesium powder which comprises mixing therewith a material capable of protecting the magnesium from combining with deleterious substances by preventing access thereof, subjecting said powder to a temperature above the melting point and below the boiling point of magnesium and to a rubbing action to cause magnesium particles to coalesce to form liquid metal and preventing access of air during said rubbing operation by providing a neutral or reducing atmosphere. 35
12. A method of treating magnesium powder which comprises mixing therewith a hydrocarbon oil, removing therefrom excess oil, and subjecting said powder to a temperature above the melting point and below the boiling point of magnesium and to a rubbing action to cause magnesium particles to coalesce to form liquid metal. 40
13. A method of treating magnesium powder which comprises subjecting the same to at least a partial vacuum, preventing access of deleterious substances and subjecting said powder to a temperature above the melting point and below the boiling point of magnesium and to a rubbing action to cause magnesium particles to coalesce to form liquid metal. 45
14. A method of treating magnesium powder which comprises subjecting the same to at least a partial vacuum, mixing therewith a material capable of protecting the magnesium from combining with deleterious substances by preventing access thereof, subjecting said powder to a temperature above the melting point and below the boiling point of magnesium and to a rubbing action to cause magnesium particles to coalesce to form liquid metal, releasing the vacuum and removing said metal. 50
15. A method of treating magnesium powder which comprises subjecting the same to at least a partial vacuum, subjecting said powder to a temperature above the melting point and below the boiling point of magnesium and to a rubbing action to cause magnesium particles to coalesce to form liquid metal, releasing the vacuum and removing said metal. 55
16. A method of treating magnesium powder which comprises subjecting the same to at least a partial vacuum, preventing access of deleterious substances and subjecting said powder to a temperature above the melting point and below the boiling point of magnesium and to a rubbing action to cause magnesium particles to coalesce to form liquid metal and condensing magnesium vapors formed in said operation. 60
17. A method of treating magnesium powder which comprises subjecting the same to at least a partial vacuum, and subjecting said powder to a temperature above the melting point and below the boiling point of magnesium and to a rubbing action to cause magnesium particles to coalesce to form liquid metal and condensing magnesium vapors formed in said operation in a condenser maintained under a partial vacuum. 65
18. A method of treating magnesium powder which comprises subjecting said powder to a temperature above the melting point and to a rubbing action to cause magnesium particles to coalesce to form liquid metal and condensing magnesium vapors formed in said operation. 70
19. A method of treating magnesium powder which comprises subjecting said powder to a temperature above the melting point and to a rubbing action to cause magnesium particles to coalesce to form liquid metal and condensing magnesium vapors formed in said operation, in the presence of a protective gas. 75
20. A method of treating magnesium powder which comprises subjecting said powder to a temperature above the melting point and below the boiling point of magnesium and to a rubbing action in the presence of an inert or reducing gas to form liquid magnesium. 80
21. A method of treating magnesium powder which comprises subjecting said powder to a temperature above the melting point and below the boiling point of magnesium and continuously moving a source of heat through said powder to sub- 85
- 90
- 95
- 100
- 105
- 110
- 115
- 120
- 125
- 130
- 135
- 140
- 145
- 150

ject the same to a rubbing action to form liquid magnesium.

22. A method of treating magnesium powder which comprises subjecting said powder to a temperature above the melting point and below the boiling point of magnesium and continuously moving a source of heat through said powder to subject the same to a rubbing action in the presence of an inert or reducing gas to form liquid magnesium.

23. A method of treating magnesium powder which comprises subjecting said powder to a temperature above the melting point and below the boiling point of magnesium and maintaining said

powder in a continuous state of agitation to form liquid magnesium, providing a reduced pressure to withdraw vapors of magnesium and condensing the same.

24. A method of treating magnesium powder which comprises subjecting said powder to a temperature above the melting point, maintaining said powder in a continuous state of agitation to subject the same to a rubbing action, the temperature and pressure being such as to cause vaporization of magnesium, removing the vapors and condensing the same.

FRANK R. KEMMER.

80

85

90

### DISCLAIMER

1,964,853.—*Frank R. Kemmer, Larchmont, N. Y. METHOD OF TREATING METAL POWDER.* Patent dated July 3, 1934. Disclaimer filed May 21, 1938, by the assignee, *Magnesium Products, Incorporated.*

Hereby enters this disclaimer to claim 24 of said patent.

[*Official Gazette June 14, 1938.*]

30

105

35

110

40

115

45

120

50

125

55

130

60

135

65

140

70

145

75

150

ject the same to a rubbing action to form liquid magnesium.

22. A method of treating magnesium powder which comprises subjecting said powder to a temperature above the melting point and below the boiling point of magnesium and continuously moving a source of heat through said powder to subject the same to a rubbing action in the presence of an inert or reducing gas to form liquid magnesium.

23. A method of treating magnesium powder which comprises subjecting said powder to a temperature above the melting point and below the boiling point of magnesium and maintaining said

powder in a continuous state of agitation to form liquid magnesium, providing a reduced pressure to withdraw vapors of magnesium and condensing the same.

24. A method of treating magnesium powder which comprises subjecting said powder to a temperature above the melting point, maintaining said powder in a continuous state of agitation to subject the same to a rubbing action, the temperature and pressure being such as to cause vaporization of magnesium, removing the vapors and condensing the same.

FRANK R. KEMMER.

80

85

90

### DISCLAIMER

1,964,853.—*Frank R. Kemmer, Larchmont, N. Y. METHOD OF TREATING METAL POWDER.* Patent dated July 3, 1934. Disclaimer filed May 21, 1938, by the assignee, *Magnesium Products, Incorporated.*

Hereby enters this disclaimer to claim 24 of said patent.

[*Official Gazette June 14, 1938.*]

30

105

35

110

40

115

45

120

50

125

55

130

60

135

65

140

70

145

75

150